

May 26, 1970

KAZURO SUZUKI ET AL

3,513,903

APPARATUS FOR CASTING INGOTS

Filed July 19, 1966

4 Sheets-Sheet 1

Fig. 1



Fig. 2



INVENTORS.  
KAZURO SUZUKI  
HIROSHI YAMAOKA  
BY  
Kurt Kelman  
AGENT

May 26, 1970

KAZURO SUZUKI ET AL

3,513,903

APPARATUS FOR CASTING INGOTS

Filed July 19, 1966

4 Sheets-Sheet 2

Fig. 3



Fig. 4



INVENTORS.  
KAZURO SUZUKI  
HIROSHI YAMAOKA  
BY  
Kurt Kelman  
AGENT

May 26, 1970

KAZURO SUZUKI ET AL

3,513,903

APPARATUS FOR CASTING INGOTS

Filed July 19, 1966

4 Sheets-Sheet 3

FIG. 5(2)



FIG. 7



FIG. 5(1)



INVENTORS:  
KAZURO SUZUKI  
HIROSHI YAMADA  
BY Kurt Kelman  
AGENT

May 26, 1970

KAZURO SUZUKI ET AL

3,513,903

APPARATUS FOR CASTING INGOTS

Filed July 19, 1966

4 Sheets-Sheet 4

*Fig. 6*

(1)



(2)

AVERAGE MAXIMUM ROUGHNESS 33  $\mu$

INVENTORS.  
KAZURO SUZUKI  
HIROSHI YAMAOKA  
BY

*Kurt Kelman*  
AGENT

1

3,513,903

APPARATUS FOR CASTING INGOTS  
Kazuro Suzuki and Hiroshi Yamaoka, Osaka-fu, Japan,  
assignors to Sumitomo Metal Industries, Ltd., Osaka,  
Japan

Filed July 19, 1966, Ser. No. 566,296

Claims priority, application Japan, July 21, 1965,  
40/43,693

Int. Cl. B22d 27/16

U.S. Cl. 164—255

2 Claims

## ABSTRACT OF THE DISCLOSURE

Ingots are cast into the cavity of an open top metallic mold. The upright mold wall has perforations and is lined by a thin permeable sand lining covering the perforations. An evacuated jacket surrounds the mold and molten metal is supplied to the bottom of the mold cavity.

This invention relates to a method for casting ingots under a gas stream and more particularly relates the casting of ingots of metals or alloys.

In general, steel or cast iron is utilized as mold material when ingots of metals or alloys are made and the mold has a long useful life. Sometimes a surface crease, crack, surface folding or blow hole is caused on the surface or in the interior of the ingot because of the high heat conductivity of the mold material and the surface lubricant used. Minor faults disappear with increasing reduction during rolling but serious faults remain after the ingots are processed to finished goods. These goods cannot be used.

An object of this invention is to provide a mold for casting ingots of metals or alloys with sound interior and sound outer surfaces in which a membrane formed by a thin sand lining is provided on the inner surface of a metallic mold to reduce the cooling speed of the surface of the ingots so that faults such as surface creases, cracks, surface folds or blow holes are prevented from appearing on the outer surface or in the interior of the ingots, and the gas generated from the membrane is exhausted outward the metallic mold.

In the prior art, such as shown in Pat. No. 3,099,052, air or an inert gas, e.g. argon, helium or nitrogen etc., is forced through the permeable material of a mold during casting, the fluid flowing outward of the mold so that no blow hole occurs.

In the present invention, the gas stream is used in a sand lined metallic mold with the same effect. Sound ingots having no blow hole, no surface crease nor crack are obtained in accordance with the present invention.

Other objects and advantages of the present invention will become readily apparent from the following detailed description of the drawing, in which:

FIGS. 1 and 2 show apparatus for casting ingots according to the present invention in respective elevational sections,

FIG. 3 is a similar view of a modified apparatus of the present invention,

FIG. 4 is a corresponding view of yet another apparatus of the present invention,

FIGS. 5(1) and (2) respectively show the surface condition of a steel ingot made in accordance with a conventional method for casting ingots using a metallic mold and the surface condition of a stainless steel ingot made in accordance with the method for casting ingots of the present invention,

FIGS. 6(1) and (2) are graphs showing the roughness of the surfaces illustrated in FIGS. 5(1) and (2), respectively, and

FIG. 7 shows a sectioned steel ingot made in a conven-

2

tional metallic mold and a sectioned alloy ingot made in accordance with the present invention, respectively.

In FIG. 1, a thin, permeable sand lining 3 (shell mold,  $\text{CO}_2$  mold) is baked to the inner surface of a heavy, perforated metallic mold 1. The holes in the mold 1 are distributed uniformly and preferably filled with non-illustrated steel wires having a melting point above 1000° C., in order to prevent entry of molten metal into the holes while permitting gas generated in the mold and a gas stream applied to the mold to be exhausted through the holes. The outside of the metallic mold 1 with the sand lining 3 is separated from the atmosphere by a vessel 8 closed by a plate member 10 made of paper or metal. The vessel 8 is partly filled with shot 9 and partly kept without filler. The bottom of the mold cavity 6 communicates with a runner 2.

The apparatus shown in FIG. 1 is operated in the following manner: while molten metal 7 is poured into the mold cavity 6 through the runner 2, the pressure in the vessel 8 is reduced by means of a non-illustrated vacuum pump. At the same time, air or an inert gas is introduced through a riser 5 and is exhausted through the sand lining 3 and the holes in the mold 1. If air or an inert gas, such as argon, helium or nitrogen is introduced, the gas generated from the sand lining during casting is carried away by the inert gas without penetrating into the molten metal. No faults due to the gas are found after the molten metal is solidified.

The apparatus of FIG. 2 is similar to the apparatus shown in FIG. 1 except for the provision of a hollow metallic mold 11 which combines the functions of the mold 1 and of the vessel 8. The operation and the effect of the apparatus shown in FIG. 2 are similar to those of the apparatus shown in FIG. 1.

In FIG. 3, a metallic mold 1, a sand lining 3, a riser 5, a mold cavity 6 and a runner 2 are similar to corresponding elements of FIG. 1. An inert gas is applied to the molten metal in mold cavity 6 from the top of the riser 5 through a pipe 12 under positive pressure. The gas generated from the sand lining 3 is driven out of the mold as explained with reference to FIG. 1.

In FIG. 4, a thin sand lining 3 is provided on the outer face of a metallic mold 1 surrounded by a vessel 8 equipped with a riser 5. Molten metal 7 is fed from a runner 2 to a mold cavity 6 between the lining 3 and the vessel 8 to form a hollow ingot. The mold 1 is exhausted by means of a vacuum pump through an exhaust pipe 13 connected thereto and gas is led from the mold cavity 6 to the exhaust pipe 13 through the sand lining 3 and the metallic mold 1. The gas generated from the sand lining 3 is exhausted out of the mold as explained in reference to FIG. 1.

The present invention was applied to the casting of ingots as follows:

## EXAMPLE 1

An 18-8 stainless steel ingot weighing 9 kg. was cast in a cast iron mold of the invention which had a diameter of 100 mm. and a height of 150 mm. The mold had 30 holes of 20 mm. diameter which were filled with sintered iron. The lining of the mold consisted of silica sand bonded with phenolic resin and was 6 mm. thick. Air was drawn into the mold at a rate of 1.2 liters per minute per  $\text{cm}^2$  by a vacuum of -180 mm. water column in the mold.

FIG. 5(1) shows the surface of the ingot so produced. FIG. 5(2) similarly shows the surface of an ingot of the same metal cast in a conventional metal mold.

As is shown in FIG. 6, the average surface roughness measured by a contact-point type instrument was  $132\mu$  maximum for the conventional ingot 1 and was  $33\mu$  maximum for the ingot 2 of the invention.

## EXAMPLE 2

A pure nickel ingot was prepared by the present invention under the following condition:

The cast iron mold employed had dimensions of 230 mm. x 100 mm. x 575 mm., and had 70 holes 50 mm. in diameter filled with sintered iron. The sand lining was 5 mm. thick, and air was drawn into the mold at a rate of 10 liters per minute per cm.<sup>2</sup> by a negative pressure of -150 mm. water column. The ingot weighed 100 kg.

Faults due to secondary shrinkage occurring at rolling 10 were eliminated by the method of the present invention.

Sections of the ingots obtained by the method of the invention (right side) under the conditions stated above and by a conventional method (left side) are shown in FIG. 7.

## EXAMPLE 3

An ingot used as raw material for 18-8 stainless steel pipe was prepared in a cast iron mold, 516 mm. x 516 mm. x 1500 mm. provided with 196 holes 86 mm. in diameter and filled with steel wire. The mold was lined with 10 mm. of chromite sand bonded with phenolic resin, and air was drawn into the mold at a flow rate of 1.6 liters per minute per cm.<sup>2</sup> by a negative pressure of 200 mm. water column in the mold. The ingot weighed 3000 kg.

Suitable lining materials include silica sand, zircon sand, chromite sand, alumina, magnesia or mixtures thereof.

The binder for the lining may be a synthetic resin, another organic material or an inorganic material. Suitable synthetic resins include phenol resin, furan resin, urea resin, polyvinyl alcohol, etc., the other organic material may be a drying oil cereal, or sodium alginate, and said inorganic material may be clay, sodium silicate, ethyl silicate, silicic acid gel etc.

As shown in the following table, the time for finishing the surface of ingots cast by the present invention is reduced to  $\frac{1}{10}$  of that needed with a conventional casting method and the yield for finished ingots is improved by 8.5%.

TABLE

|                                                   | Conven- | Method of |
|---------------------------------------------------|---------|-----------|
|                                                   | tional  | present   |
|                                                   | method  | invention |
| Time for preparing surface of ingots in hours.... | 3.0     | 0.3       |
| Yield for finished ingots in percent.....         | 86.5    | 95.0      |

## What we claim is:

1. An apparatus for casting ingots comprising:

- (a) a unitary self-sustaining metallic mold member having an outer upright face and an inner upright face, said mold member being formed with a plurality of openings therethrough between said faces, said inner face bounding a mold cavity having an open top and communicating with the atmosphere through said top;
- (b) a permeable sand lining covering said inner face and said openings, the thickness of said sand lining being much smaller than the thickness of said mold member between said faces thereof;
- (c) a vessel enveloping said outer face and defining a substantially closed space with said outer face;
- (d) means for evacuating said space and for thereby drawing a gas stream from said mold cavity through said lining and said openings; and
- (e) supply means other than said open top for supplying molten metal to a portion of said mold cavity below said openings.

2. An apparatus as set forth in claim 1, wherein said supply means include a runner having an orifice in said cavity below said openings.

## References Cited

## UNITED STATES PATENTS

|           |         |                       |           |
|-----------|---------|-----------------------|-----------|
| 315,741   | 4/1885  | Henderson -----       | 164—120   |
| 3,006,046 | 10/1961 | Shephard et al. ----- | 164—16    |
| 3,098,268 | 7/1963  | Zifferer -----        | 164—16    |
| 3,099,868 | 8/1963  | Grott -----           | 164—16    |
| 3,099,052 | 7/1963  | Suzuki et al. -----   | 164—66    |
| 3,222,735 | 12/1965 | Sylvester -----       | 164—306 X |
| 2,991,267 | 7/1961  | Bean -----            | 260—38    |
| 863,733   | 8/1907  | Lustig -----          | 164—66    |
| 3,210,810 | 10/1965 | Potter -----          | 164—12 X  |
| 1,544,592 | 7/1925  | Murray -----          | 249—114 X |
| 2,997,756 | 8/1961  | Strom -----           | 164—255 X |
| 2,379,401 | 6/1945  | Poulter -----         | 164—255 X |
| 2,489,322 | 11/1949 | Olsen et al. -----    | 249—141 X |
| 783,576   | 2/1905  | Haggenjos -----       | 164—410   |
| 1,855,529 | 4/1932  | Poe -----             | 249—114   |
| 1,585,391 | 5/1926  | Kubota -----          | 249—114 X |
| 2,312,796 | 3/1943  | Campbell -----        | 164—255   |

J. SPENCER OVERHOLSER, Primary Examiner

V. RISING, Assistant Examiner

## U.S. CL. X.R.

164—62, 66, 138, 366, 410; 113, 114, 141, 174; 249—204